

No. 738,703.

Patented September 8, 1903.

# UNITED STATES PATENT OFFICE.

GOTTFRIED SCHMALFUSS, OF COLOGNE, GERMANY, ASSIGNOR OF ONE-HALF TO HENRY LIERZ, OF PHILADELPHIA, PENNSYLVANIA.

## ADHESIVE TABLET.

SPECIFICATION forming part of Letters Patent No. 738,703, dated September 8, 1903.

Application filed August 28, 1902. Serial No. 121,393. (No model.)

*To all whom it may concern:*

Be it known that I, GOTTFRIED SCHMALFUSS, a subject of the King of Prussia, German Emperor, residing at Cologne-on-the-Rhine, in the Province of the Rhine, Kingdom of Prussia, German Empire, have invented an Improved Adhesive Tablet, of which the following is a specification.

My invention relates to improvements in adhesive tablets adapted for use as a substitute for liquid glue and other liquid adhesives; and it consists in an adhesive tablet comprising powdered dextrine and powdered sugar mixed and compressed while dry, as hereinafter described.

Dextrine, gum-arabic, or a similar adhesive substance in form of powder is to be mixed dry with sugar or soap powder or any other material in form of powder being conducive to its solubility, and then by pressing this mixture it is brought into a handy solid shape, square or rectangular tablets answering the purpose. I thus produce a tablet composed of a powdered adhesive substance and a powdered substance of quicker solubility, which while associated intimately with each other and commingled remain mechanically sepa-

rated, so that each preserves its identity, the same being mixed and compressed while dry.

By the term "tablet" as used in this specification I mean a cake, stick, or other form adapted to be readily handled and used and of any desired shape and size.

These tablets show a granular structure and they are not subject to excessive hardening, bending, or becoming split. If part of the surface is wetted with a brush, an immediate solution of a certain part of this adhesive substance will take place, so that it may be used in the same way as any other ordinary liquid glue, but all disadvantages being eliminated.

What I claim as my invention, and desire to secure by Letters Patent of the United States, is—

An adhesive tablet comprising powdered dextrine and powdered sugar, mixed and compressed while dry, substantially as described.

In testimony whereof I have signed my name to this specification in the presence of two subscribing witnesses.

GOTTFRIED SCHMALFUSS.

Witnesses:

CHARLES LESIMPLE,  
CARL SCHMITT.